



US006794010B1

(12) **United States Patent**  
Yamaguchi et al.

(10) Patent No.: **US 6,794,010 B1**  
(45) Date of Patent: **Sep. 21, 2004**

(54) **CARPET, STAINPROOFING AGENT FOR CARPET AND METHOD FOR TREATING THE CARPET**

(75) Inventors: **Fumihiko Yamaguchi**, Settsu (JP); **Masamichi Morita**, Settsu (JP); **Yasushi Nakamae**, Settsu (JP); **Hiroko Yano**, Settsu (JP); **Kazuyuki Satoh**, Settsu (JP); **Masato Ioki**, Settsu (JP)

(73) Assignee: **Daikin Industries, Ltd.**, Osaka (JP)

(\*) Notice: Subject to any disclaimer, the term of this patent is extended or adjusted under 35 U.S.C. 154(b) by 0 days.

(21) Appl. No.: **09/368,429**

(22) Filed: **Aug. 5, 1999**

(30) **Foreign Application Priority Data**

Aug. 18, 1998 (JP) ..... 10-232084  
Apr. 20, 1999 (JP) ..... 11-111737

(51) **Int. Cl.** <sup>7</sup> ..... **D05C 17/00**

(52) **U.S. Cl.** ..... **428/96; 428/97; 524/458;**  
526/245

(58) **Field of Search** ..... 428/97, 96; 524/458;  
526/245

(56) **References Cited**

U.S. PATENT DOCUMENTS

3,594,353 A 7/1971 Domba  
3,819,772 A 6/1974 Kolobow  
4,592,940 A \* 6/1986 Blyth et al. ..... 252/8.62  
4,636,331 A 1/1987 Sako et al.

|             |          |                             |
|-------------|----------|-----------------------------|
| 4,835,300 A | 5/1989   | Fukui et al.                |
| 4,868,042 A | 9/1989   | Adiletta                    |
| 5,143,991 A | * 9/1992 | Amimoto et al. .... 526/245 |
| 5,316,850 A | * 5/1994 | Sargent et al. .... 428/96  |
| 5,349,003 A | 9/1994   | Kato et al.                 |
| 5,614,123 A | 3/1997   | Kubo et al.                 |
| 5,630,846 A | 5/1997   | Hara et al.                 |
| 5,830,963 A | 11/1998  | Kubo et al.                 |
| 5,843,328 A | 12/1998  | Pacifci et al.              |
| 5,883,175 A | 3/1999   | Kubo et al.                 |

OTHER PUBLICATIONS

JP 59-150175 English Translation.\*

JP 5910175A, Aug. 28, 1984, English Abstract.\*

\* cited by examiner

*Primary Examiner*—Cheryl A. Juska

*Assistant Examiner*—Jenna-Leigh Befumo

(74) *Attorney, Agent, or Firm*—Birch, Stewart, Kolasch & Birch, LLP

(57)

**ABSTRACT**

The relates to a carpet comprising a stainproof-treated textile, wherein the carpet has stainproof ratio (%) of at least 30% as defined below:

$$\text{Stainproof ratio (\%)} = 100 \times (\Delta E_N - \Delta E_{Tn}) / \Delta E_N$$

$\Delta E_N$ : Color difference after stainproof test of untreated carpet;

$\Delta E_{Tn}$ : Color difference after stainproof test of carpet treated by the stainproof agent;

n: the number of cleaning; cleaning is conducted according to AATCC-138, n≤20.

**7 Claims, No Drawings**



between said fluorine-containing stainproofing agent comprising Rf-containing compound and carpet pile, and also hardens coating:



wherein R<sup>1</sup> to R<sup>6</sup> are the same or different, and represent —H, —OH, —CH<sub>2</sub>OCH<sub>3</sub>, —CH<sub>2</sub>OH, —CH<sub>2</sub>CH<sub>2</sub>OH, —CH<sub>2</sub>CH<sub>2</sub>CH<sub>2</sub>OH, or —CH<sub>2</sub>OC<sub>2</sub>H<sub>5</sub>, preferably —CH<sub>2</sub>OH.

As crosslinking agent represented by formula (1), trimethylolmelamine and hexamethylolmelamine are particularly preferable. Example of commercial name of the crosslinking agent is SUMITEX RESIN M-3 (trimethylolmelamine; SUMITOMO CHEMICAL Co. LTD.).

Coating mass of the triazine ring-containing compound preferably ranges from 0.01 to 1.0% by weight based on the unit weight of carpet. When coating mass is less than 0.01% by weight, cleaning durability is insufficient. When coating mass is more than 1.0% by weight, cleaning durability is not improved but results in hard feeling, thereby not preferable.

Catalyst is preferably added to the triazine ring-containing compound to accelerate a reaction. Examples of catalyst are formic acid, acetic acid and like organic carboxylic acids; organic carboxylates between the organic carboxylic acids and ammonium, sodium, potassium, etc.; sulfuric acid, persulfuric acid, hydrochloric acid, phosphoric acid, nitric acid and like inorganic acids; inorganic acid salts between the inorganic acids and ammonium, sodium, potassium, magnesium, zinc, aluminum, iron, etc. The amount of catalyst is not specifically limited to, but usually 5–100% by weight based on the amount of triazine ring-containing compound.

The stainproofing agent for carpet may be in the form of aqueous dispersion or solution in a solvent.

The stainproofing agent of the present invention can be applied by any method according to the kind of the material to be treated. For example, there can be used a method for applying the agent of the invention on the surface of material to be treated, using a known application procedure such as immersion, coating, etc., followed by drying. Furthermore, the stainproofing agent of the present invention may further comprise additives and a crosslinking agent other than said crosslinking agent. For example, polymethyl methacrylate/ethyl methacrylate (P-MMA/EMA) and like polymer, additives such as insect repellents, flame retardants, antistatic agents, dye fixing agents, wrinkle inhibitors, softeners and stain block agents which inhibit adhesion of acid dye may be appropriately added.

The material to be treated with the stainproofing agent of the present invention is preferably a textile, in particular, a carpet. Examples of the textile are animal-origin natural fibers such as cotton, hemp, wool, silk, etc.; synthetic fibers such as polyamide (nylon), polyester, polyvinyl alcohol, polyacrylonitrile, polyvinyl chloride, polypropylene, etc.; semisynthetic fibers such as rayon, cellulose acetate, etc.; inorganic fibers such as glass fibers, carbon fibers, asbestos fibers, etc.; and a mixture of these fibers. Preferable fibers are polyamide (nylon), polyester, polyvinyl alcohol, polyacrylonitrile, polyvinyl chloride, polypropylene and like synthetic fibers, rayon, cellulose acetate and like semisynthetic fibers or a mixture thereof. The textile may be in any form such as a fiber, a yarn, a cloth and the like. When a

carpet is treated with the stainproofing agent of the present invention, the carpet may be formed after treating fibers or yarns with the stainproofing agent. Alternatively, the formed carpet may be treated with the stainproofing agent.

The carpet of the invention may be pre-treated with stain block agent before stainproof treatment. Examples of stain block agent are generally a poly(meth)acrylic acid and a sulphonate acid-containing phenol/formaldehyde condensation product, specifically FX-668F (Minnesota Mining and Manufacturing Co.), SR-300 (E.I. du Pont de Nemours and Company). The stain block agent is preferably used in a sufficient amount which allow 0.05–10% by weight of active ingredient based on the weight of carpet to be adhered on carpet. Stain block agent may be applied according to a usual treatment process such as hot air treatment, steam treatment, boiled water treatment, etc.

The stainproofing agent of the invention may further comprises PEG and/or a copolymer comprising

- (1) at least one selected from polyoxyethylene chain-containing acrylate and methacrylate; and
- (2) at least one reactive monomer selected from glycerol methacrylate and glycidyl methacrylate).

The copolymer or PEG may be used in an amount of 1–50% by weight, preferably 2–20% by weight based on the solid content of repellent.

Color of carpet to be treated includes blue.

With respect to color of carpet,

L=40 to 80, preferably L=40 to 60;

a=+0.1 to −0.8, preferably a=−0.1 to −0.6;

b=−13 to −25, preferably b=−17 to −21.

The carpet of the invention maintains a stainproof degree during resoiling of at least 20%, preferably at least 30% after one cycle of contamination, cleaning and recontamination.

#### BEST MODE FOR CARRYING OUT THE INVENTION

The invention is described below in detail by way of example. However, the invention is in no way limited to the examples.

Evaluation procedures of water-repellency, oil-repellency and stainproof property, and cleaning process are shown below.

##### <Water-repellency>

Five drops of isopropanol/water mixture having the following composition are slowly placed on the surface of carpet textile. Water repellency is represented by a maximum score at which at least 4 drops maintain a liquid form (repellent) after 3 minutes.

TABLE 1

|    | Composition (% by volume) |             |       |
|----|---------------------------|-------------|-------|
|    | Score                     | Isopropanol | Water |
| 55 | 0                         | 0           | 100   |
|    | 2                         | 2           | 98    |
|    | 5                         | 5           | 95    |
|    | 10                        | 10          | 90    |
|    | 15                        | 15          | 85    |
|    | 20                        | 20          | 80    |
|    | 25                        | 25          | 75    |
| 60 | 30                        | 30          | 70    |
|    | 40                        | 40          | 60    |
|    | 50                        | 50          | 50    |

##### <Oil-repellency>

According to AATCC-TM-118-1966, five drops of the following test solution are slowly placed on the surface of carpet. Penetration state of the drops are observed after 3

minutes. Oil-repellency is represented by a maximum score at which at least 4 drops show no penetration into carpet.

TABLE 2

| Score | Test solution                                                                 | Surface tension<br>(mN/m: 25° C.) |
|-------|-------------------------------------------------------------------------------|-----------------------------------|
| 0     | Inferior to 1                                                                 |                                   |
| 1     | Nujol                                                                         | 31.2                              |
| 2     | A mixture of N-hexadecane (35 parts by weight) and Nujol (65 parts by weight) | 29.6                              |
| 3     | n-hexadecane                                                                  | 27.3                              |
| 4     | n-tetradecane                                                                 | 26.7                              |

## &lt;Stainproof Property Test 1&gt;

Carpet treated with a stainproofing agent is evaluated according to AATCC-123-1995.

Carpet textile is cut into a 5.5 cm×8 cm test piece. The test piece is allowed to stand in thermohygrostat (21° C., 65% RH) for 4 hours, dried sufficiently, followed by contaminated with a dry soil having the following composition. Specifically, five carpet test pieces are attached to a ball mill in such a manner that the stainproof surface of the carpet is in a upward direction. 0.031 g of dry soil per 1 cm<sup>2</sup> surface area of the carpet test piece (corresponding to 6.82 g in case of five carpet test pieces) and 50 ceramic balls (2.0 cm in diameter) are put in the ball mill. The ball mill is then rotated at 80 rpm for 7.5 minutes to give the carpet test piece on the surface of which the dry soil is uniformly adhered. The ball mill has a tubular shape, and a base inner diameter of 12.0 cm and a height of 9.5 cm. The excessive dry soil on the carpet test piece is thoroughly removed by aspiration with domestic vacuum cleaner. Color difference ( $\Delta E$ ) on the surface of carpet is determined with color difference meter (MINOLTA CR-310). Stainproof ratio (%) is calculated on the basis of the following equation.

$$\text{Stainproof ratio (\%)} = 100 \times (\Delta E_N - \Delta E_{Tn}) / \Delta E_N$$

$\Delta E_N$ : Color difference after stainproof test of untreated carpet

$\Delta E_{Tn}$ : Color difference after stainproof test of carpet treated by the stainproof agent

n: the number of cleaning.

Dry soil composition, L, a and b values are shown below:

| Composition  | Content (% by weight) |
|--------------|-----------------------|
| Peat moss    | 38.4                  |
| Cement       | 18                    |
| Kaoline      | 18                    |
| Silica       | 18                    |
| Carbon black | 1.15                  |
| Iron oxide   | 0.3                   |
| Nujol        | 6.25                  |

with respect to Lab values, L: 25–31, a: 2.3–2.6, b: 4.2–4.8.

## &lt;Stainproof Property Test 2&gt;

<Stainproof property test 2> is evaluated in the same manner as <Stainproof property test 1> except that the size of carpet textile is 11 cm×8 cm; and that the amount of dry soil per 1 cm<sup>2</sup> surface area of the carpet test piece is 0.0062 g (corresponding to 1.64 g in case of three carpet test pieces); and that rotation conditions are 80 rpm for 5 min.

## &lt;Cleaning Method&gt;

Stated more specifically:

- (i) the surface of carpet test piece (11 cm×11 cm) is washed with running water (50° C.) for 1 min, followed by squeezed with mangle (pressure: 5 mg/cm<sup>2</sup>).

(ii) The carpet test piece is fixed and set on the testing stand of cleaning test machine (STAIN & CLEANING TESTER: YOSHIDA SEIKI SEISAKUSYO) as defined in JIS L1023-1992 in order that rotary brushes rub carpet piles.

(iii) Cleaning of the carpet is carried out by pouring 4.1 ml of 1% sodium lauryl sulfate (SLS) aqueous solution (adjusted at pH 8 with NaOH aqueous solution) warmed to 50° C. to carpet with pipette, followed by rotating rotary brush and testing stand.

One cleaning is composed of 5 rotations in regular direction, 5 rotations in reverse direction, further 5 rotations in regular direction and 5 rotations in reverse direction during which rotary brushes maintain rubbing carpet.

15 “Cleaning three times” mean that the process is repeated 3 times except that SLS 1% aqueous solution is not further added.

16 “Cleaning five times” means that the process is repeated 5 times except that SLS 1% aqueous solution is not added.

20 The number of revolutions of the testing stand is 20 rpm. The number of rotation of brush is 240 rpm. Vacuum and water jet nozzle of cleaning test machine are not used.

25 The carpet is thoroughly rinsed with running water (50° C.), squeezed with mangle, and then dried in hot-air drying chamber at 105° C. for 30 min leading to completion of cleaning.

## EXAMPLE 1

30 Nylon 6,6 carpet textile (cut pile, pile density: 40 oz/yd<sup>2</sup>, pile height: 1/4 inch, color: light blue) was dipped in water, squeezed with mangle to adjust wet pickup (the increased weight, represented by % by weight, of carpet after dipping in comparison with initial weight of carpet test piece) at 20% by weight.

35 A Stainproofing agent composition as shown in table 4 was prepared by mixing and stirring 8 parts by weight of UNIDYNE TG-3010 (Rf group-containing stainproofing agent for carpet; DAIKIN INDUSTRIES LTD.), 1.9 parts by weight of SUMITECH RESIN M-3 (trimethylolmelamine: SUMITOMO CHEMICAL CO., LTD.), 0.6 part by weight of SUMITECH ACCELERATOR (ACX; catalyst for SUMITECH RESIN M-3 which is a product of SUMITOMO CHEMICAL Co., LTD.) and 89.5 parts by weight of water.

40 The carpet test piece (20 g) was treated with the stainproofing agent composition (1.5 g; corresponding to 400 ppm fluorine atom per 1 g of carpet), followed by heat-treated with pin stenter at 130° C. for 10 min.

45 The carpet test piece was cleaned (1 time, 3 times, 5 times) according to the above-defined method to evaluate water-repellency, oil-repellency and stainproof property before and after cleaning. The results are shown in table 6.

## EXAMPLES 2–6

50 Stainproofing agent compositions as shown in table 4 were prepared. The carpet test piece was treated in the same manner as example 1.

The results are shown in table 6.

## EXAMPLE 7

55 A stainproofing agent composition was prepared by diluting 6 parts by weight of emulsion (solid content 30% by weight) comprising Rf-maleate/methylmethacrylate (MMA)=60/40 (weight ratio) copolymer, SUMITEX RESIN M-3 and SUMITEX ACCELERATOR (ACX) with 94 parts by weight of water. The carpet test piece was treated

with the stainproofing agent composition thus obtained in the same manner as example 1.



wherein n is an integer of 3 to 8.

#### EXAMPLES 8-10

The carpet test piece shown in example 1 was subjected to stain block processing. To a stain block agent (FX-668F: Minnesota Mining and Manufacturing Co.) diluted to 0.7% with water was added MgSO<sub>4</sub> (1%), and pH of the solution was adjusted at 2 with sulfamic acid. The carpet test piece was boiled in the solution for 5 minutes. The test piece was washed with running water to remove an excess stain block agent and dried at 130° C. The resulting carpet test piece was dipped in water, squeezed with mangle to adjust wet pickup thereof at 20%.

Stainproofing agents as shown in table 4 were prepared to treat the carpet test piece in the same manner as example 1. The results are shown in table 6.

A stain block agent is a treatment applied to a material in order to inhibit adhesion of acid dye in the process of stainproof processing of carpet.

#### COMPARATIVE EXAMPLES 1-4

Stainproofing agent mixtures shown in table 5 were prepared and used for treating the carpet test piece in the same manner as example 1. The results are shown in table 6.

TABLE 4

| Rf-containing Stainproofing Agent Kind/Amount Ex. (Wt. Part) | Crosslinking Agent Kind/Amount (Wt. Part) | Water (Wt. part) | Other Additives Kind/Amount (Wt. Part) |
|--------------------------------------------------------------|-------------------------------------------|------------------|----------------------------------------|
| 1 UNIDYNE TG3010/8                                           | SUMITEX RESIN M-3/1.8                     | 89.5             | ACX (0.6)                              |
| 2 UNIDYNE TG3010/8                                           | SUMITEX RESIN M-3/0.9                     | 89.8             | ACX (0.3)                              |
| 3 Rf-maleate-MMA Copolymer 30% Emulsion/5                    | SUMITEX RESIN M-3/0.9                     | 93.8             | ACX (0.3)                              |
| 4 SCOT GUARD FX-1373M/5                                      | SUMITEX RESIN M-3/0.9                     | 93.8             | ACX (0.3)                              |
| 5 SCOT GUARD FX-1367F/8                                      | SUMITEX RESIN M-3/2.1                     | 89.2             | ACX (0.7)                              |
| 6 N-140/5                                                    | SUMITEX RESIN M-3/1.5                     | 93               | ACX (0.5)                              |
| 8 UNIDYNE TG3010/8                                           | SUMITEX RESIN M-3/1.8                     | 89.8             | ACX (0.3)                              |
| 9 Rf-maleate-MMA Copolymer 30% Emulsion/5                    | SUMITEX RESIN M-3/0.9                     | 93.8             | ACX (0.3)                              |

TABLE 4-continued

| 5  | Rf-containing Stainproofing Agent Kind/Amount Ex. (Wt. Part) | Crosslinking Agent Kind/Amount (Wt. Part) | Water (Wt. part) | Other Additives Kind/Amount (Wt. Part) |
|----|--------------------------------------------------------------|-------------------------------------------|------------------|----------------------------------------|
| 10 | 10 SCOT GUARD FX-1367F/8                                     | SUMITEX RESIN M-3/2.1                     | 89.2             | ACX (0.7)                              |

TABLE 5

| 15 | Rf-containing Stainproofing Agent Kind/Amount Ex. (Wt. Part) | Crosslinking Agent Kind/Amount (Wt. Part) | Water (Wt. part) | Other Additives Kind/Amount (Wt. Part) |
|----|--------------------------------------------------------------|-------------------------------------------|------------------|----------------------------------------|
| 20 | 1 UNIDYNE TG3010/8                                           | — / —                                     | 89.5             | —                                      |
| 2  | 2 Rf-maleate-MMA Copolymer 30% Emulsion/5                    | — / —                                     | 89.8             | —                                      |
| 25 | 3 Rf-maleate-MMA Copolymer 30% Emulsion/5                    | ELASTRON BN-69/1.5                        | 93.35            | Cat64 (0.15)                           |
| 4  | 4 SCOT GUARD FX-1367F/5                                      | — / —                                     | 93.8             | —                                      |

TABLE 6

| 30          | Number of Cleaning | Water-Repellency (Score) |    |    |   | Oil-Repellency (Score) |   |   |   | Stainproof Ratio (%) |    |    |    |
|-------------|--------------------|--------------------------|----|----|---|------------------------|---|---|---|----------------------|----|----|----|
|             |                    | 0                        | 1  | 3  | 5 | 0                      | 1 | 3 | 5 | 0                    | 1  | 3  | 5  |
| Example 1   | 20                 | 15                       | 15 | 15 | 0 | 0                      | 0 | 0 | 0 | 41                   | 39 | 37 | 35 |
| Example 2   | 20                 | 15                       | 10 | 10 | 0 | 0                      | 0 | 0 | 0 | 41                   | 38 | 35 | 33 |
| Example 3   | 20                 | 20                       | 15 | 15 | 0 | 0                      | 0 | 0 | 0 | 42                   | 40 | 38 | 35 |
| Example 4   | 20                 | 20                       | 15 | 15 | 0 | 0                      | 0 | 0 | 0 | 40                   | 39 | 38 | 36 |
| Example 5   | 25                 | 25                       | 25 | 20 | 1 | 1                      | 1 | 1 | 1 | 50                   | 49 | 47 | 43 |
| Example 6   | 25                 | 20                       | 20 | 15 | 0 | 0                      | 0 | 0 | 0 | 52                   | 50 | 48 | 45 |
| Example 7   | 20                 | 15                       | 15 | 10 | 0 | 0                      | 0 | 0 | 0 | 40                   | 38 | 37 | 32 |
| Example 8   | 25                 | 15                       | 15 | 10 | 0 | 0                      | 0 | 0 | 0 | 55                   | 54 | 51 | 49 |
| Example 9   | 30                 | 25                       | 20 | 20 | 0 | 0                      | 0 | 0 | 0 | 55                   | 55 | 54 | 54 |
| Example 10  | 30                 | 25                       | 20 | 20 | 1 | 1                      | 1 | 1 | 1 | 55                   | 55 | 54 | 54 |
| Comp. Ex. 1 | 20                 | 0                        | x  | x  | 0 | 0                      | 0 | 0 | 0 | 43                   | 28 | 18 | 15 |
| Comp. Ex. 2 | 20                 | 15                       | 0  | 0  | 0 | 0                      | 0 | 0 | 0 | 41                   | 27 | 21 | 18 |
| Comp. Ex. 3 | 20                 | 15                       | 5  | 5  | 0 | 0                      | 0 | 0 | 0 | 27                   | 26 | 25 | 24 |
| Comp. Ex. 4 | 10                 | 5                        | x  | x  | 1 | 1                      | 1 | 0 | 0 | 33                   | 28 | 22 | 15 |

In table 3, the number of cleaning "0" means before cleaning.

50 With respect to stainproof ratio, carpet which is not treated with a stainproofing agent has a stainproof ratio of 100% before contamination and 0% after contamination.

#### EXAMPLE 11

55 Stain block processing was carried out in advance in the same manner as examples 8-10.

A stainproofing agent composition was prepared by mixing 8 parts by weight of TG-3010, 0.9 part by weight of SUMITEX RESIN M-3, 0.3 part by weight of SUMITEX ACCELERATOR, 0.7 part by weight of polyethyleneglycolmethacrylate(PEGMA)/glycerol methacrylate(GMA)=70/30 (by weight ratio) copolymer and 90.1 parts by weight of water. The carpet test piece was treated by the composition in the same manner as example 1.

60 The test piece was subjected to a test cycle comprising <stainproof property 2>, cleaning and <stainproof property

## 9

2>. After the last <stainproof property 2> treatment, stainproof ratio of the test piece was determined. The results are shown in table 8.

## COMPARATIVE EXAMPLE 5

Stain block processing was carried out in advance in the same manner as examples 8–10.

A stainproofing agent composition as shown in table 7 was prepared. The carpet test piece was treated with the stainproofing agent composition in the same manner as example 1. The test piece was subjected to the evaluation test as shown in example 11. The results are shown in table 8.

TABLE 7

| Rf-Containing Stain-proofing Agent Kind/Amount (Wt. Part) | Crosslinking Agent Kind/Amount (Wt. Part) | PEGMA/GMA Copolymer (Wt. Part) | Water (Wt. Part) | Other Additive Kind/Amount (Wt. Part) |
|-----------------------------------------------------------|-------------------------------------------|--------------------------------|------------------|---------------------------------------|
| Ex. 11 UNIDYNE TG3010/8                                   | SUMITEX RESIN M-3/0.9                     | 0.7                            | 90.1             | ACX (0.3)                             |
| Comp. UNIDYNE TG3010/8                                    | — / —                                     | — / —                          | 92               | — / —                                 |
| Ex. 5                                                     |                                           |                                |                  |                                       |

TABLE 8

| Stainproof ratio (%) |         |                 |
|----------------------|---------|-----------------|
|                      | Initial | Recontamination |
| Ex. 11               | 65      | 35              |
| Comp. Ex. 5          | 60      | 15              |

What is claimed is:

1. A carpet comprising a stainproof-treated textile, wherein the carpet has a stainproof ratio defined below of at least 30%:

$$\text{Stainproof ratio (\%)} = 100 \times (\Delta E_N - \Delta E_{Tn})/E_N, \text{ wherein}$$

$\Delta E_N$  is the color difference after a stainproof test of untreated carpet;

$\Delta E_{Tn}$  is the color difference after a stainproof test of carpet treated by the stainproof agent; and

n is the number of cleanings conducted according to 45 AATCC-138 and  $n \leq 20$ ;

wherein the carpet is treated with a stainproofing agent composition for carpet consisting essentially of:

(1) a fluorine-containing stainproofing agent consisting essentially of a fluoroalkyl-containing compound; and (2) a triazine ring-containing crosslinking agent represented by formula (1)



wherein  $\text{R}^1$  to  $\text{R}^6$  are the same or different and represent —H, —OH, —CH<sub>2</sub>OCH<sub>3</sub>, —CH<sub>2</sub>OH, —CH<sub>2</sub>CH<sub>2</sub>OH, —CH<sub>2</sub>CH<sub>2</sub>CH<sub>2</sub>OH, or CH<sub>2</sub>OCH<sub>2</sub>H<sub>5</sub>; and

(3) at least one of a catalyst and an additive, wherein the catalyst is selected from the group consisting of organic carboxylic acids; organic carboxylates

## 10

between the organic carboxylic acids and ammonium, sodium, or potassium; inorganic acids; inorganic acid salts between the inorganic acids and ammonium, sodium, potassium, magnesium, zinc, aluminum, or iron; and

wherein the additive is selected from the group consisting of insect repellents, flame retardants, antistatic agents, dye fixing agents, wrinkle inhibitors, softeners and stain block agents which inhibit adhesion of acid dye.

2. The carpet according to claim 1 wherein the carpet maintain stainproof ratio of at least 30% after five times of cleaning.

3. The carpet according to claim 1 wherein the fluorine-containing stainproofing agent consisting essentially of a

25 fluoroalkyl-containing compound has at least one member selected from the group consisting of fluoroalkyl-containing maleic acid diester copolymer, fluoroalkyl-containing adipic acid diester compound and fluoroalkyl-containing urethane compound.

30 4. The carpet according to claim 1 which is blue with L=40 to 80; a=+0.1 to -0.8; and b=-13 to -25.

5. The carpet according to claim 1 which maintains a stainproof ratio of at least 20% after recontamination when the carpet is subjected to a test cycle of contamination, cleaning and recontamination.

35 6. A carpet treated with a stainproofing agent composition, consisting essentially of:

(1) a fluorine-containing stainproofing agent consisting essentially of a fluoroalkyl-containing compound and (2) a triazine ring-containing crosslinking agent represented by formula (1)



wherein  $\text{R}^1$  to  $\text{R}^6$  are the same or different and represent —H, —OH, —CH<sub>2</sub>OCH<sub>3</sub>, —CH<sub>2</sub>OH, —CH<sub>2</sub>CH<sub>2</sub>OH, —CH<sub>2</sub>CH<sub>2</sub>CH<sub>2</sub>OH, or CH<sub>2</sub>OCH<sub>2</sub>H<sub>5</sub>.

7. A carpet treated with a stainproofing agent composition, which consists essentially of

(1) a fluorine-containing stainproofing agent consisting essentially of a fluoroalkyl-containing compound and

(2) a triazine ring-containing crosslinking agent, and at least one of PEG and a copolymer consisting essentially of:

(3) at least one monomer selected from the group consisting of acrylate having a polyoxyethylene chain and methacrylate having a polyoxyethylene chain; and

(4) at least one reactive monomer selected from the group consisting of glycerol methacrylate and glycidyl methacrylate.

\* \* \* \* \*